

# United States Patent

[11] 3,570,772

[72] Inventors **Robert Ben Booth**  
Stamford, Conn.;  
**Herman Hartjens, Ridgewood, N.J.; John**  
**Joseph Falvey, Noroton Heights, Conn.**  
[21] Appl. No. **852,504**  
[22] Filed **Aug. 22, 1969**  
[45] Patented **Mar. 16, 1971**  
[73] Assignee **American Cyanamid Company**  
Stamford, Conn.  
Continuation-in-part of application Ser. No.  
**617,069, Feb. 20, 1967, now abandoned.**

---

[54] **DI(4-5 CARBON BRANCHED PRIMARY ALKYL DITHIOPHOSPHATE PROMOTERS FOR THE FLOTATION OF COPPER MIDDLEINGS**  
**7 Claims, No Drawings**

[52] U.S. Cl. .... **241/24,**  
209/10, 209/166, 241/29

[51] Int. Cl. .... **B02c 11/00,**  
B03d 1/02, B03d 1/08

[50] **Field of Search**..... 209/166,  
167, 3, 10; 241/20, 24, 29

[56] **References Cited**  
UNITED STATES PATENTS  
2,664,199 12/1953 Barkev ..... 209/167  
3,086,653 4/1963 Booth ..... 209/166

*Primary Examiner*—Tim R. Miles  
*Assistant Examiner*—Robert Halper  
*Attorney*—Samuel Branch Walker

---

**ABSTRACT:** In the flotation of copper sulfides, diisobutyl dithiophosphates, diisoamyl dithiophosphates and di(2-methyl-1-butyl) dithiophosphates give a superior flotation rate, recovery and selectivity as compared with conventional dialkyl dithiophosphates, often permitting a coarser grind, and flotation of middlings, followed by a regrind ultimately resulting in a higher recovery of copper.

DI(4-5 CARBON BRANCHED PRIMARY ALKYL)  
DITHIOPHOSPHATE PROMOTERS FOR THE  
FLOTATION OF COPPER MIDLINGS

## CROSS REFERENCES

This application is a continuation-in-part of our application Ser. No. 617,069, filed Feb. 20, 1967, which is a continuation-in-part of our application Ser. No. 535,001, filed Mar. 17, 1966, both now abandoned in favor of this application.

This invention relates to the beneficiation of sulfide ores for the recovery of copper values occurring therein; more particularly to a process of flotation in which a sulfide ore is floated in the presence of a compound which in aqueous solution ionizes to give a dialkyl dithiophosphate ion of the formula:



where R is a branched chain primary alkyl group of not more than 5 carbon atoms. With less than 4 carbons, a primary alkyl group cannot be branched. For purposes of convenience, these compounds are referred to as di(4-5 carbon branched primary alkyl) dithiophosphates. This includes the diisobutyl dithiophosphates, the diisoamyl dithiophosphates and the di(2-methyl-1-butyl) dithiophosphates.

The promoter may be added as the free acid or as a salt such as the ammonium or sodium or potassium or calcium salt. The material may be added either in pure form as a solid or liquid, as the case may be, or mixed with excess alkalies such as sodium or potassium carbonates to give a dry powder; or as aqueous solutions.

Even when classed as a sulfide ore there may be some of the metal values present as an oxide or an appreciable part of the metal may be present as the oxide or in various oxidized forms. The sulfide ores are generally beneficiated by crushing, and then grinding the ore to obtain a pulp; usually the grinding is wet grinding. A flotation promoter may be added either after the grinding or in the wet grinding step. Frequently the promoter is added in the wet grinding step to aid in uniform distribution. A frothing agent or other additives may be added and the ore is then aerated to produce a froth at the surface of the pulp, either by mechanical agitation while adding air, or by aeration alone. The metal values adhere to the bubbles in the froth and are floated off from the surface of the aerated pulp. Such promoters are sometimes called collectors.

Such flotation operations are well known in the industry. U.S. Pat. No. 1,593,232, F. T. Whitworth "Art of Concentrating of Mineral Ores by Flotation," Jul. 20, 1926, describes the reaction product of phosphorous pentasulfide with cresylic acid as a promoter. U.S. Pat. No. 2,038,400, F. T. Whitworth, "Flotation Reagent," Apr. 21, 1936, describes the reaction product of phosphorus pentasulfide with aliphatic alcohols. This patent shows the formula:



This patent does not refer to these compounds as diaryl or dialkyl dithiophosphates but such are proper names for them.

Among such dithiophosphates which have been sold commercially are the diethyl, the diisopropyl, the di-sec-butyl, dihexyl and dicresyl. These materials have been used alone and in combination and have been added as the free acid, the sodium, potassium and ammonium salts.

Diisobutyl dithiophosphoric acid and its nickel salt are referred to in the text "Organic Phosphorus Compounds" Gennady M. Kosolapoff, John Wiley & Sons, Inc., New York, 1950 at page 253. A method of preparing is disclosed on page 236 as a general method.

It has now been found surprisingly that the di(4-5 carbon branched primary alkyl) dithiophosphates as the sodium, potassium, ammonium and calcium salts and including the dithiophosphoric acid itself, and mixtures thereof, are particularly useful as flotation promoters particularly if the ore to be floated contains middling particles which result from coarse grinding or from intimate association of the component minerals which make up the ore. The latter type of middlings frequently exist even after fine grinding.

10 Middling particles thus are composed of two or more, and often several, mineral species. Such polyphase particles are generally more difficult to concentrate by flotation than free mineral grains.

15 A. M. Gaudin, in the text, "Flotation," McGraw Hill Book Company, Inc., New York, 1957, in Chapter 13, pages 393 to 413, gives an excellent description of middling particles, and the problems and economics involved in their treatment by flotation. While some ores are free-milling ores, that is, the

20 values are readily separated from the gangue by crushing and grinding to permit the application of flotation techniques, other ores present a middling treatment problem which in the past has been difficult to solve and in many cases has not been solved adequately to date. The extractive metallurgist is

25 forced to compromise between obtaining a desired high recovery of mineral values and the grade of the concentrate produced. High recoveries in concentrates of low grade entail high treatment costs in subsequent upgrading and refining operations, which may force the rejection of larger percentages of the contained metal values so as to obtain a concentrate which is salable or amenable to further treatments. Also in many cases, the middling particles are not recovered, even though amenable to standard refining processes, and thus represent high losses of the desired mineral values.

30 35 The di(4-5 carbon branched primary alkyl) dithiophosphate promoters described in this invention provide a means of solving this middling treatment problem. The compounds can be given other names; for example, the diisobutyl compound is also named 0,0-diisobutyl phosphorodithioate. This nomenclature is currently used by Chemical Abstracts and indexed under "isobutyl."

Any theory of action is, of course, somewhat speculative and the applicants do not wish to be bound by the correctness

45 of such theory but observations appear to be consistent with the theory that the di(4-5 carbon branched primary alkyl) dithiophosphates have branched methyl groups on the ends of the alkyl chains, which improve the floatative efficiency of the overall promoter molecule.

50 55 The phosphorus-bearing promoter, bonds to the surface of the ore particles and the alkyl groups are in a better position to impart hydrophobicity to the ore particles and to enhance their collection by the bubbles of the froth. Also the possibility exists that the branching of the organic radicals in the structure of the promoter enhances the interaction of the promoter on the surface of the mineral surface and the frother molecule on the bubble surface, which serves to improve the collection of mineral particles, particularly difficultly floatable middling particles.

60 65 Whether such theories are correct or speculative, it is found that a coarser grinding gives good recovery as if only a comparatively small portion of the metal sulfides are exposed, still the present promoters are powerful enough to cause particles having such mineral value to float. Hence, a much coarser grind may be used, without loss of values to the rougher tailings, permitting a major reduction in the grinding costs.

Some ores are fairly readily ground; others are less amenable toward grinding; so that fine grinding involves considerable power, time and equipment and is costly. It is found that by

70 75 using the present di(4-5 carbon branched primary alkyl) dithiophosphates, larger particles having a smaller proportion of sulfide ore value may be floated and as a result rougher concentrate or first float is obtained containing a larger percentage of the total mineral values than has been possible with prior art procedures.

The middlings, in this rougher concentrate, may be then reground and thus only a comparatively small portion of the total quantity of ore must be reground to separate the mineral values from the gangue. A secondary, cleaner float may then be made in which the ore values are separated from any gangue as the particles are then all fairly small, the valuable particles of ore have less gangue attached, and a high grade of concentrate is obtained.

As the cost of grinding ores such as copper, lead, zinc, cobalt, nickel, molybdenum and cadmium, and mixtures thereof, is an appreciable and important part of the milling cost, the reduction in grinding requirements without loss of grade or value in the final product is an advantage. Usually it is found that there is less loss in the flotation tailings than with the more conventional promoters which have been previously used. Even though the losses in the tailings are usually only of the order of 5-20 percent of the values in the ore, reduction in these losses is extremely important. Large copper operations, for instance, may mine as much as 50,000 tons of ore a day. A small percentage increase in recovery which may be accomplished without additional costs is of great economic value.

As set forth in the examples, certain prior art examples are used by way of comparisons. The average major ore is treated by practices which are the result of years of experimentation and practical experience. The average mill is continually experimenting toward developing a flotation system or flowsheet which is more economical. In many mills any improvement which can be unequivocally identified by analysis is regarded as a tremendous advantage. In most mills, improvements which can only be detected by statistical analysis are sufficient for management to switch from one promoter and/or flowsheet, to another promoter and/or flowsheet. In a large mill, it is not uncommon to have a fair size fraction of a mill, from 10 percent for one-half, so designed that it may be operated under somewhat varied condition so as to show comparable operating costs on a major scale in plant operations. The results obtained by such comparisons are carefully studied, and in many instances an experimental period of running is necessary so that analytical errors can balance out and not conceal trace improvements. Thus, it can be seen that any change will show up by analysis as an improvement will immediately be incorporated in the mill flowsheet. Even changes which show such a slight improvement that comparison of results on side-by-side operation on major scales for a month are needed to show there is in fact an improvement are considered extremely important. Some major mills have pilot plants which can handle large daily tonnages of ore, which are used primarily for checking on any possibility of improvement of flowsheets.

The form in which the present novel promoter is added is usually not critical. It may be added as the free acid, a salt with sodium, calcium, ammonium, or as a mixture of the sodium salt with alkalies such as sodium carbonate and potassium carbonate or as a solution in water. The shipping convenience, and facility of handling and measuring is importantly affected by the physical form, and the preferred form may vary from mill to mill depending on transportation facilities and metering and feeding equipment. The promoter is usually added after the grinding operation, for maximum effectiveness, and thoroughly mixed with the ore. As water is present, and the quantity of promoter is small, it is most unlikely that the ion that was originally associated with the promoter has any effect on the system, and the acid and various salt forms give generally similar results.

In contrast, the nature of the alkyl group can have a critical effect on optimum efficiency. As shown in the examples below, the di(4-5 carbon branched primary alkyl) dithiophosphates have a much improved action over conventional dithiophosphates.

Diisobutyl dithiophosphoric acid can be produced by the reaction of diisobutyl alcohol in the ratio of 4 moles to 1 mole of phosphorus pentasulfide by changing the alcohol to the

reactor and adding the phosphorus pentasulfide in increments. Temperatures from a normal room temperature of about 20° C. up to about 50° C. give good and rapid reaction. At lower temperatures, the reaction becomes undesirably slow. At higher temperatures, the alcohol can volatilize, or by-products form. After the reaction is completed, unreacted phosphorus pentasulfide and solid impurities may be filtered from the liquid obtained, which is diisobutyl dithiophosphoric acid. Even with commercial grades of alcohol and phosphorus pentasulfide an excellent promoter is obtained. The free acid is conveniently taken up in a hydrocarbon solvent such as heptane or petroleum ether, and ammonia added to precipitate out the ammonium salt; or the free acid may be reacted with sodium carbonate and/or potassium carbonate to form the sodium and potassium salts, or mixtures. Such reaction methods are conventional in the preparation of other esters of dithiophosphoric acid.

The alcohols used as starting materials are:



Mixtures of these alcohols may be used, so that the substituents on any one phosphorus are not necessarily the same.

Another way to describe the alcohols is by the formula:



40 where  $m$  is 1 or 2, and  $n$  is 1 or 0, and the sum of  $n$  and  $m$  is 1 or 2.

Mixtures of the promoters of the present invention are effective in attaining high recovery of metal values. Such mixtures may be prepared by blending dry promoters together and using the resulting mixture in flotation operations. Alternately mixed promoters may be prepared by known methods by reacting mixtures of alcohols with phosphorus pentasulfide. The resulting reaction products are compounds in which the alkoxy groups attached to any one phosphorus may be the same or different.

Manufacturing procedures which have been used with other alcohols may be conveniently used with the present alcohols, or mixtures thereof. As the details of such procedures are well known further description appears unnecessary here.

Certain specific aspects of the present invention are set forth in more detail in the following examples in which all parts are by weight unless otherwise specified.

55 60 65 Operations are carried out at ambient temperatures in the mill which may range from slightly above freezing in the winter to temperatures of a hot summer day without deleterious effect on operating procedures. The temperature, where significant, is set forth in detail. All parts are by weight, unless otherwise stated.

#### EXAMPLE 1

A Norwegian copper ore (about 2.00 percent Cu) containing chalcopyrite and pyrite in a graphitic silicate gangue, was ground with 5.0 lb./ton hydrated lime and conditioned for 2 minutes with 0.6 lb./ton yellow corn dextrose to control the flotation of graphite and 0.060 lb./ton of a 6-8 carbon atom alcohol as frother. Sodium diisobutyl dithiophosphate, 0.025 lb./ton, was added as copper promoter and agitated with the

ore pulp for 2 minutes. Flotation was conducted for 8 minutes with two further additions of the diisobutyl dithiophosphate promoter of 0.0125 lb./ton each. A copper concentrate was removed, which contained 21.42 percent Cu in 9.00 percent of the total weight of the flotation feed and represented a recovery of 96.69 percent of the total copper.

In a second flotation test, on this ore, the identical procedure was followed except that sodium dissecondarybutyl dithiophosphate was used as copper promoter and the frother requirement was higher, 0.108 lb./ton. The copper recovery was 87.39 percent in a concentrate which assayed 19.62 percent Cu and represented 8.44 percent of the total weight of the flotation feed.

The above metallurgical results demonstrate that the diisobutyl dithiophosphate promoter of the present invention

time was 7 minutes, the frother was 0.09 pounds per ton of ore of pine oil. Flotation was carried out in a laboratory Fagergren flotation machine. With the above constant, tests were carried out using ammonium diisobutyl dithiophosphate at a dosage of 0.05 pounds per ton. For comparison a collector B was chosen consisting of 0.018 pounds per ton isopropyl ethyl thionocarbamate and 0.04 pounds per ton of sodium isopropyl xanthate.

This combination had been found to produce the highest copper recovery on this particular ore after evaluation of all available commercial collectors prior to development of the present diisobutyl dithiophosphate and represents the highest skill of a competitive art.

Comparative results at two different grinding levels are as follows:

| Test No.: | Grind, percent +65M | Collector                                | Calculated feed, percent Cu | Concentrate, percent Cu | Tailing, percent Cu | Percent recovery Cu |
|-----------|---------------------|------------------------------------------|-----------------------------|-------------------------|---------------------|---------------------|
| 30/31     | 11.0                | "B"                                      | 1.65                        | 20.20                   | 0.228               | 87.2                |
| 32/33     | 11.0                | Diisobutyl dithio phosphate <sup>1</sup> | 1.68                        | 20.01                   | 0.214               | 88.2                |
| 34/35     | 24.4                | "B"                                      | 1.62                        | 18.52                   | 0.250               | 85.8                |
| 36/37     | 24.4                | Diisobutyl dithio phosphate <sup>1</sup> | 1.64                        | 16.68                   | 0.210               | 88.4                |

<sup>1</sup> As the ammonium salt.

was more effective than the dissecondarybutyl dithiophosphate promoter and required less frother to achieve flotation of the copper. The latter promoter is used currently in many commercial copper flotation operations.

#### EXAMPLE 2

The same ore as used in example 1 also was employed in two additional flotation tests. The procedure was identical to that used in example 1 except that in the first test 0.050 lb./ton diisoamyl dithiophosphate as promoter and 0.084 lb./ton alcohol frother were used. The copper recovery was 96.55 percent in a concentrate assaying 13.55 percent Cu.

In the second test, 0.05 lb./ton of mixed di-primary-amyl dithiophosphate, as described in U.S. Pat. No. 3,068,653 was employed as promoter. In the test, the frother requirement was higher, 0.096 lb./ton. The copper recovery was 95.62 percent in a concentrate assaying 16.78 percent Cu. Thus, the diisoamyl dithiophosphate promoter of the present invention was more effective than the mixed di-primary-amyl dithiophosphate as described in the prior test. The high recovery and low grade show the remarkable pulling power on middlings.

#### EXAMPLE 3

A Canadian copper ore (1.45 percent Cu) was ground to minus 100 mesh in the presence of 1.6 lb./ton hydrated lime, 0.05 lb./ton sodium cyanide, and 0.1 lb./ton zinc sulfate. The ore pulp was conditioned for 2 minutes with 0.06 lb./ton methylisobutyl carbinol as frother and 0.02 lb./ton mixed sodium-potassium diisoamyl dithiophosphate as promoter. Flotation was conducted for 4 minutes and resulted in the recovery of 93.9 percent of the copper in a concentrate assaying 20.44 percent Cu and representing 6.65 percent of the weight of the ore.

25 The tailings produced in the first two tests were screened and the fractions analyzed for copper. The results of these two analyses are shown below. It can be seen that in all size fractions above 150 mesh, the tailings produced with diisobutyl dithiophosphate had less copper than with the standard collector B. As no free copper mineral was found in the size fractions larger than 150 mesh, it is concluded that the lower tailings produced with ammonium diisobutyl dithiophosphate was due to its superior ability to float middling particles of copper sulfide which contain both copper sulfide and gangue.

| Screen size, Tyler Mesh | Rougher tailing, 30/31 diisobutyl dithiophosphate, percent Cu | Rougher tailing, 32/33 Collector "B", percent Cu |
|-------------------------|---------------------------------------------------------------|--------------------------------------------------|
| +65                     | 0.34                                                          | 0.40                                             |
| -65 +100                | 0.13                                                          | 0.21                                             |
| -100 +150               | 0.13                                                          | 0.15                                             |
| -150 +200               | 0.14                                                          | 0.14                                             |
| -200                    | 0.20                                                          | 0.20                                             |

30 It is to be noted that the results were particularly spectacular on both the -65 + 100 and the +65 mesh product. These particles had both copper values and gangue, which had not been broken apart by grinding operations.

#### EXAMPLE 5

35 This test on a second South American copper ore shows that the additional recovery with diisobutyl dithiophosphate as the promoter is maintained after the cleaner flotation without sacrificing grade of final concentrate. The comparison was again between ammonium diisobutyl dithiophosphate and the collector B of example 1. This collector is in regular use on the flotation of this ore.

| Collector                               | Calculated feed, Percent Cu | Rougher concentration, Percent Cu | Cleaner concentration, Percent Cu | Percent recovery |
|-----------------------------------------|-----------------------------|-----------------------------------|-----------------------------------|------------------|
| Diisobutyl dithiophosphate <sup>1</sup> | 1.77                        | 26.41                             | 52.42                             | 88.7             |
| "B"                                     | 1.83                        | 24.45                             | 47.07                             | 87.1             |

<sup>1</sup> As the ammonium salt.

#### EXAMPLE 4

Samples of a South American copper ore were ground to -28 mesh, that is, all the material would pass a 28 mesh screen. As is common in grinding size practice, the amount retained of other mesh sizes is as given below.

Comparative tests were conducted using the same coarse grinds at an alkalinity of pH 10.7, adjusted with lime. Flotation

70 75 The collector dosage was the same as in example 4. The frother was pine oil at 0.05 pounds per ton. The alkalinity was at pH 11 maintained with lime. This test is indicative of results on a fully integrated pilot plant operated at 1,000 pounds per hour of copper ore. At this particular plant when calculated for full operation, the additional copper recovery has a value of about \$3,000 per day.

It is also to be noted that the cleaner concentrate has a higher grade which reduces smelting problems.

#### EXAMPLE 6

Two other copper ores, designated Ore No. 1 and Ore No. 2, were chosen. These ores assayed 1.37 percent copper and 1.56 percent Cu respectively. Comparative tests were carried out with several collectors. The grind was -28 mesh with 19 percent +65 mesh; alkalinity was adjusted to pH 10.5 with lime; promoter dosage was 0.05 pounds per ton. The frother with the No. 1 ore was 0.05 pounds per ton of a polyglycol and for the No. 2 ore pine oil at 0.08 pounds per ton. Flotation times were respectively 5 and 7 minutes. For each ore all variables other than the promoter were maintained constant. The average of closely similar results from tests conducted in duplicate were as follows:

| Promoter                         | Copper    | Copper    | Rougher | tailing | Percent | Percent | Rougher | tailing | Percent | Percent | Recovery |
|----------------------------------|-----------|-----------|---------|---------|---------|---------|---------|---------|---------|---------|----------|
|                                  | Ore No. 1 | Ore No. 2 |         |         |         |         |         |         |         |         |          |
|                                  |           |           |         |         |         |         |         |         |         |         |          |
| Isobutyl DTP <sup>1</sup>        | 0.238     | 0.380     |         |         |         |         |         |         |         |         |          |
| Secondary butyl DTP <sup>1</sup> | 0.256     | 0.435     |         |         |         |         |         |         |         |         |          |
| n-Butyl DTP <sup>1</sup>         | 0.256     | 0.438     |         |         |         |         |         |         |         |         |          |

<sup>1</sup> Dithiophosphate, as the ammonium salt.

The copper content of the rougher flotation tailings represents a loss in copper values and this is a critical factor in determining the efficiency of a promoter in the flotation process.

The figures look particularly impressive when calculated out as the recovery of additional copper on a large-scale operation—with no additional operating or capital costs. The reduction in copper loss in the above examples corresponds to 0.36 lb. and 1.1 lb. of copper per ton or ore treated, which at large operations treating 10 million tons of ore or more per year correspond to an additional copper recovery of 3,600,000 to 11,000,000 lbs. of copper per year. The value of the collector or promoter is great in relation to its cost, which in view of the raw materials used in the manufacture of the dithiophosphates would be nominal as compared with the market in value of copper recovered.

#### EXAMPLE 7

Samples of Ore No. 2, as described in example 6, are ground and floated by the method and with lime and frother as described in example 6. As flotation promoter, diisobutyl dithiophosphates in the form of the free acid, the sodium, potassium, and mixed sodium potassium salts, the sodium salt with a large excess of soda ash, and the calcium salt were used on separate representative portions of the ore. The flotation tailings were assayed for copper and the results of the tests were analogous to those obtained with the ammonium salt in example 6 as indicated in the following summary.

| Promoter:                                                 | Percent Cu in rougher tailing |
|-----------------------------------------------------------|-------------------------------|
| Ammonium salt <sup>1</sup>                                | 0.380                         |
| Sodium salt (technical grade)                             | 0.380                         |
| Potassium salt                                            | 0.384                         |
| Mixed sodium-potassium salts                              | 0.385                         |
| Sodium salt with excess sodium carbonate<br>50% by weight | 0.380                         |
| Sodium salt prepared as a 40% aqueous solution            | 0.387                         |
| Calcium salt prepared as 20% aqueous solution             | 0.390                         |
| Free acid                                                 | 0.385                         |

<sup>1</sup> From Example 6.

#### EXAMPLE 8

A lead-zinc ore containing zinc sulfide, partly finely disseminated in iron sulfide and gangue with considerable middling present even at a fine grind of 70 percent minus 200 mesh and 100 percent through 65 mesh, is subjected to

rougher flotation with the conventional collector for that ore, namely, isopropyl xanthate, at 0.31 pounds per ton of ore and ammonium diisobutyl dithiophosphate at 0.07 pounds per ton of ore, under otherwise identical conditions using a pine oil frother at 0.04 pounds per ton. The feed material was tailing from a lead flotation step. Lime was added to adjust the pH to 10.2 and copper sulfate added for sphalerite activation at 2.0 pounds per ton. Better recoveries and higher grade concentrates were obtained due to the better middling recovery and greater selectivity towards the iron sulfide. Test results were as follows:

| Collector                               | Rougher concentration |            | Rougher tailing |            | Recovery |      |
|-----------------------------------------|-----------------------|------------|-----------------|------------|----------|------|
|                                         | Percent Zn            | Percent Fe | Percent Zn      | Percent Fe | Zn       | Fe   |
| Isopropyl xanthate                      | 33.3                  | 19.6       | 3.0             | 28.0       | 72.8     | 14.4 |
| Diisobutylidithiophosphate <sup>1</sup> | 42.8                  | 14.0       | 2.0             | 28.6       | 82.0     | 9.5  |

<sup>1</sup> As the ammonium salt.

This table shows a spectacular drop in the percentage of zinc lost in the rougher tailings. The corresponding improved recovery of zinc shows up in the recovery percentages, the grade is much improved. In such a recovery operation the iron is regarded as a contaminant. The improvement in the grade of the zinc product through the reduction of the iron content in the rougher concentrate is an advantage in the use of the diisopropyl dithiophosphate promoter.

Whereas in the above examples, the advantages are primarily set forth from the standpoint of an improved recovery of a purer copper under conditions which are otherwise the same, advantages of the present flotation reagents can be in part utilized towards (1) a higher recovery of copper or (2) towards copper recoveries of an improved grade in the concentrate or (3) towards a higher flotation rate permitting the treatment of larger tonnages in given mill equipment of ore with a recovery equivalent to that using conventional reagents or (4) a greater selectivity towards iron sulfide to reduce smelter expenses or (5) a decrease in the cost of grinding; or in part all of these. In commercial operations, the flowsheet can be modified towards an increased output of copper by forcing the grinding and flotation units, and accepting a lower grade and lower recovery, or the recovery of copper in quantity or grade can be optimized. The factors involved vary from time to time even in the same mill depending on the economic position of the market as regards both price and demand for copper, and other variables. It will be understood by those most skilled in the art that with the superior promoters here taught, the chief engineer will modify the flowsheet to optimize production under the particular conditions controlling at the time of operation.

The applicability of the novel promoters for zinc, copper-nickel, copper-cobalt, and silver ores is similar. It would unduly extend the length of this specification to give complete details of all of the conditions in all ores under which advantages are found.

Promoters other than the diisobutyl dithiophosphate are shown in the following examples in which, to avoid unduly lengthening the description, comparative data is given in tabular form.

#### EXAMPLE 9

Under conditions otherwise controlled and kept the same, comparative runs were made on two different copper ores, using five carbon alkyls in the dialkyl dithiophosphates (DTP). These are shown in the following table:

|                      | Copper recovery    |                   |
|----------------------|--------------------|-------------------|
|                      | Chile ore, percent | Utah ore, percent |
| Di(primary amyl) DTP | 86.6               | 85.1              |
| Di(2-methyl-1-butyl) | 87.3               | 85.2              |
| Di(3-methyl-1-butyl) | 87.9               | 85.7              |

## EXAMPLE 10

For a particular Arizona ore a thionocarbamate promoter has been standard, being chosen by mill operators with years of experience attempting to use the most economically advantageous promoter of which they were aware for the particular ore.

Whereas the increase from 78.7 to 84.3 or 85.3 percent of copper recovered does not appear to be too large, when it is considered that the extra copper is recovered at no additional cost, effectively, and that operations at a major mill can run in the neighborhood of 10 million tons of ore a year, it can be seen that the economical value of this recovery would run into several millions of dollars worth of copper per year.

The results tabulated are:

## CHALCOPYRITE ORE FROM ARIZONA

| Collector, lb./ton    | Concen-<br>tration,<br>percent<br>Cu | Recovery                   |               |                               |
|-----------------------|--------------------------------------|----------------------------|---------------|-------------------------------|
|                       |                                      | Tailings,<br>percent<br>Cu | Cu<br>percent | MoS <sub>2</sub> ,<br>lb./ton |
| Thionocarbamate, 0.02 | 25.15                                | 0.220                      | 78.7          | 0.51                          |
| Diisobutyl DTP, 0.02  | 24.34                                | 0.159                      | 84.3          | 0.59                          |
| Diisoamyl DTP, 0.02   | 24.64                                | 0.151                      | 85.3          | 0.57                          |

## EXAMPLE II

Similar runs were made on a chalcocite ore from Chile as shown in the following table:

| Chalcocite ore from Chile, lb./ton    | Concen-<br>tration,<br>percent<br>Cu | Recovery                  |               |                                          |
|---------------------------------------|--------------------------------------|---------------------------|---------------|------------------------------------------|
|                                       |                                      | Tailing,<br>percent<br>Cu | Cu<br>percent | MoS <sub>2</sub> ,<br>percent<br>lb./ton |
| Thionocarbamate, 0.018+               |                                      |                           |               |                                          |
| Na-isopropyl xanthate, 0.4 (Standard) | 17.04                                | 0.331                     | 77.58         | 0.42                                     |
| Diisoamyl DTP, 0.05                   | 18.86                                | 0.316                     | 77.93         | 0.42                                     |
| Diisobutyl DTP, 0.05                  | 15.98                                | 0.305                     | 79.42         | 0.43                                     |

Again the standard collector is the one which has been used at this mill based on years of experience and is to be taken as representative of the best that those skilled in the art can achieve.

## EXAMPLE 12

A run was made on a South American copper ore with all other variables the same other than the promoters. The mill report being:

|                       | Collectors                                            |                  |                                    |                        |                       |
|-----------------------|-------------------------------------------------------|------------------|------------------------------------|------------------------|-----------------------|
|                       | Thiono-<br>carbamate<br>plus<br>isopropyl<br>xanthate | Amyl<br>xanthate | Di(sec-<br>ondary<br>butyl)<br>DTP | Diiso-<br>butyl<br>DTP | Diiso-<br>amyl<br>DTP |
| Cu percent recovery:  |                                                       |                  |                                    |                        |                       |
| After 2 min.          | 66.9                                                  | 53.5             | 66.7                               | 69.1                   | 72.5                  |
| After 4 min.          | 74.2                                                  | 70.9             | 73.7                               | 75.1                   | 78.0                  |
| After 7 min.          | 77.6                                                  | 77.6             | 77.3                               | 77.9                   | 79.4                  |
| Cu Grade Total        | 17.0                                                  | 16.1             | 19.0                               | 18.0                   | 16.0                  |
| Fe recovery, lb./ton: |                                                       |                  |                                    |                        |                       |
| After 2 min.          | 14.2                                                  | 7.9              | 7.9                                | 8.7                    | 11.0                  |
| After 4 min.          | 15.7                                                  | 12.2             | 9.3                                | 9.9                    | 12.0                  |
| After 7 min.          | 16.6                                                  | 14.2             | 10.3                               | 10.7                   | 12.3                  |

## NOTE.—Procedure:

Grind 19.5% plus 65 mesh with lime to give pH=11.0 in flotation.

Condition 1 minute with 0.05 lb./ton collector.

1° float 2 minutes with 0.05 lb./ton collector.

2° float 2 minutes with 0.05 lb./ton collector.

3° float 3 minutes with 0.05 lb./ton collector.

## EXAMPLE 13

Using the conditions otherwise the same, a mill report on a copper ore from Canada is as follows:

## Procedure:

Grind to 4 percent +65 mesh

Condition 1 minute with 0.045 lb./ton of collector and 0.048 lb./ton of alcohol frother at pH 8.5

|                                | Collector             |                        |                       |
|--------------------------------|-----------------------|------------------------|-----------------------|
|                                | Isopropyl<br>xanthate | Diiso-<br>butyl<br>DTP | Diiso-<br>amyl<br>DTP |
| Cu recovery:                   |                       |                        |                       |
| After 1 min.                   | 54.0                  | 64.9                   | 76.4                  |
| After 3 min.                   | 79.1                  | 80.6                   | 86.2                  |
| After 6 min.                   | 87.2                  | 86.3                   | 89.4                  |
| Conc., total, grade percent Cu | 21.8                  | 19.8                   | 19.8                  |

## EXAMPLE 14

In this example, the objective was to demonstrate the relative performance of the various alkyl dithiophosphates made from 5 carbon atom alcohols. The procedure in all tests was the same and consisted of grinding to a fineness of 19.3 percent +65 mesh, adding lime to the grinding step to produce a pH 10.7 in subsequent flotation. The ore was then conditioned with 0.045 lb./ton of promoter and 0.095 lb./ton of a frothing agent and floated for consecutive periods of 1, 2 and 4 minutes. The results of these tests were as follows:

|  | Percent Cu recovery:   | Di-n-<br>amyl<br>DTP | Di(iso-<br>amyl)<br>DTP | Di(2-<br>methyl-<br>1-butyl)<br>DTP |
|--|------------------------|----------------------|-------------------------|-------------------------------------|
|  |                        | After 1 min.         | 70.7                    | 71.2                                |
|  | After 3 min.           | 13.6                 | 14.4                    | 14.4                                |
|  | After 7 min.           | 2.3                  | 2.4                     | 2.3                                 |
|  | Percent total recovery | 86.6                 | 88.0                    | 87.3                                |

The increase in rate of recovery and the increase in total recovery are important.

It is to be noted that the increase in recovery in effect is copper recovered without additional cost.

As most flotation operations are conducted at a pH of between about 9 and about 11 and usually 10 or 11, the form in which the di(4-5 carbon branched primary alkyl) dithiophosphate is added is relatively immaterial and even if the di(4-5 carbon branched primary alkyl) dithiophosphate is blended with fairly large quantities of alkalies or other carriers to aid in its handling characteristics, such alkalies are present in too small a quantity to have a significant effect on the pH of the operation. The di(4-5 carbon branched primary alkyl) dithiophosphate could be used in a flotation circuit which operates on the acid side of neutral and still give effective flotation, but the above results are given as representing

facts more closely in accordance with accepted practices in ore processing.

Obviously the flotation may be accomplished in one or more stages, or separately for sands and slimes, in accordance with conventional practice for promoters. The present promoter gives improved results even if blended in part with conventional promoters. The quantities illustrated by example are representative of best results with particular ores. Im-

proved results can be obtained with these di(4-5 carbon branched primary alkyl) dithiophosphate promoters over a range of about 0.01 to 0.3 pounds per ton of ore, depending on ore grade, size of grind, and milling conditions. The most advantageous results are most often around 0.05 lb./ton of ore.

We claim:

1. A process of beneficiating copper ores by froth flotation of an ore pulp, in which a significant part of the ore is present in the rougher flotation as middlings, with a particle size of larger than 150 mesh, with many of such larger particles consisting of more than one mineral species, at least one of which is gangue in the presence of a flotation promoter to recover copper values in said ore, the improvement wherein the promoter consists essentially of a dithiophosphate of the formula



where each R is a branched chain primary alkyl group of not more than 5 carbon atoms selected from the group consisting of isobutyl, isoamyl and 2-methyl-1-butyl, with the R's not necessarily the same and Me is a dissociating cation selected

from the group consisting of hydrogen, sodium, ammonium, potassium and calcium.

2. The process of claim 1 in which from about 0.01 to about 0.3 pound of diisobutyl dithiophosphate per ton of ore is used as the promoter.

3. The process of claim 2 in which at least 10 percent of the ore in the initial flotation is larger than 65 mesh, and the concentrate from the flotation step is reground, and subjected to an additional flotation step.

4. The process of claim 1 in which from about 0.01 to about 0.3 pound of diisoamyl dithiophosphate per ton of ore is used as the promoter.

5. The process of claim 4 in which at least 10 percent of the ore in the initial flotation is larger than 65 mesh, and the concentrate from the flotation step is reground, and subjected to an additional flotation step.

6. The process of claim 1 in which from about 0.01 to about 0.3 pound of di(2-methyl-1-butyl) dithiophosphate is used as the promoter.

7. The process of claim 6 in which at least 10 percent of the ore in the initial flotation is larger than 65 mesh, and the concentrate from the flotation step is reground, and subjected to an additional flotation step.

25

30

35

40

45

50

55

60

65

70

75

UNITED STATES PATENT OFFICE  
CERTIFICATE OF CORRECTION

Patent No. 3,570,772 Dated March 16, 1971

Inventor(s) Robert Ben Booth, Hermen Hartjens & John Joseph

It is certified that error appears in the above-identified patent and that said Letters Patent are hereby corrected as shown below:

Column 1, line 12 after "particularly" omit -- to --.

Column 3, line 49 "or ore" should read -- of ore --.

Column 3, line 75 "changing" should read -- charging --.

Column 4, line 32 "-methyl" should read -- 2-methyl --.

Column 7, line 34 "or" should read -- of --.

Column 8, line 61 "date" should read -- data --.

Column 9, line 35 "0.4" should read -- 0.04 --.

Signed and sealed this 18th day of April 1972.

(SEAL)

Attest:

EDWARD M. FLETCHER, JR.  
Attesting Officer

ROBERT GOTTSCHALK  
Commissioner of Patents